

## UNITED STATES PATENT OFFICE

2,287,049

SURFACE TREATMENT OF MAGNESIUM AND  
MAGNESIUM BASE ALLOYS

Mike A. Miller, New Kensington, Pa., assignor to  
Aluminum Company of America, Pittsburgh,  
Pa., a corporation of Pennsylvania

No Drawing. Application July 8, 1941,  
Serial No. 401,463

6 Claims. (Cl. 148—8)

This invention relates to the cleaning of magnesium articles and is more particularly concerned with the production of bright surfaces upon articles of that metal and its alloys.

The term "magnesium" as used in this specification and in the appended claims includes not only magnesium itself but also the so-called magnesium base alloys containing more than 70 per cent magnesium.

During the working of magnesium and its alloys, the metal usually becomes coated with foreign matter, such as the lubricant used during the working operation and various other impurities, which may even be embedded in the surface of the metal itself. This foreign matter usually may be removed by etching the surface of the work piece in any of several chemical solutions, the most generally used of which are aqueous solutions containing sulfuric acid. These chemical treatments, however, are not entirely satisfactory. One of their chief disadvantages is that, while they remove foreign matter and clean the surface of the metal in a satisfactory manner, they generally accompany the cleaning of the surface with a dull rough etch. This necessitates a subsequent operation if the surface of the metal is to be smoothed and brightened.

An object of this invention, then, is to provide an improved method for cleaning articles of magnesium. A more particular object is to devise such a method which also provides the magnesium work piece with a bright shiny surface.

The specific object of this invention is to provide a method whereby surfaces of magnesium objects may be treated in an aqueous cleaning solution containing sulfuric acid to remove lubricants and other foreign matter, with which the surface of the metal has become contaminated during a working or similar operation, and at the same time be rendered bright and shiny.

My invention is predicated upon the discovery that if the aqueous sulfuric acid solutions heretofore used for cleaning magnesium surfaces also contain certain soluble organic aromatic compounds, the action of these cleaning solutions upon the magnesium becomes modified and, instead of leaving the magnesium surface dull and rough, the cleaning action of the solutions upon the metal is accompanied by a brightening effect which leaves the metal uniformly bright and shiny.

The soluble additive substances which are used with sulfuric acid to modify the action of the cleaning solution in accordance with my invention are the soluble organic compounds compris-

ing the group consisting of phenol, resorcinol, pyrogallol, and gallic acid. These substances are all aromatic compounds, and they may be considered to be aromatic hydroxy compounds since phenol, resorcinol, and pyrogallol are constructed with one or more hydroxyl groups upon a single benzene ring, and gallic acid is similarly constructed with the hydroxyl groups upon its benzene ring predominating in number over the carboxyl group and thereby causing gallic acid to behave like these other organic compounds. Also, I have found that the organic content used to modify the action of the solution need not be restricted to a single one of these compounds but may consist of mixtures of these substances. While it is preferable to use these aromatic compounds, it is possible to substitute their salts, such as their alkali metal and ammonium salts, since such salts form these free aromatic compounds in the aqueous sulfuric acid solution.

The total amount of these aromatic additive compounds in the solution may range from about 0.5 per cent to about 15 per cent by weight, but is preferably maintained between about 3 per cent and 5 per cent. Such amounts of these aromatic compounds in aqueous solutions containing between about 1 and 10 per cent, and preferably between about 2 and 6 per cent by weight sulfuric acid cause the surface of magnesium, which becomes dull when cleaned in the known sulfuric acid solutions, to become not only freed of any foreign matter but also bright and shiny. The balance of the cleaning solution is substantially all water. By this I mean that the balance of the solution, while it may contain magnesium sulfate and other reaction products produced during the cleaning operation and minor amounts of other substances which do not interfere with the cleaning and brightening action of the sulfuric acid and the aromatic additive compounds, is essentially aqueous. This aqueous solution also may contain one or more of the aliphatic polybasic acids from the group consisting of oxalic, malic, citric, and tartaric acids which comprise another group of substances which are in many respects similar to these aliphatic additive compounds and are more fully described in my copending application, Serial No. 401,464, filed July 8, 1941. The presence of these aliphatic dibasic acids, however, is not necessary since they do not appear to influence the cleaning and brightening effect of the solution.

These aromatic additive compounds do not appear to interfere with the cleaning action of the sulfuric acid to any substantial extent. Their

function seems to be restricted almost entirely to modifying the action of the solution in such a way that the magnesium work piece becomes bright and shiny during the cleaning step. It seems likely, however, that the phenolic compounds in the solution serve to retard slightly the attack of the sulfuric acid and to make its action more uniform. This is not objectionable; in fact, it may be desirable, since the retarded and uniform attack of the acid prevents "wedge effect," i. e. the progressively diminishing cross section sometimes produced upon elongated articles of magnesium when the acid attack is greater upon some parts of the article immersed in the solution than upon other parts.

Preferably the solution should be maintained at about room temperature during the cleaning operation. Higher temperatures may also be employed; and use of the cleaning solution at higher temperatures may be desirable in some cases, since then smaller amounts of the active agents generally are needed, and the cleaning and brightening step may be accelerated by heating the solution. However, the more rapid action at elevated temperatures may result in the presence of a greater amount of acid spray, and therefore be objectionable.

By the treatment of magnesium articles in accordance with my invention, hydrocarbons, such as lubricating oil, and other foreign matter are removed from the surface of the work piece. The cleaning solution also attacks the surface of the metal itself and dissolves away any oxide and other magnesium compounds which may have formed upon the surface; and in addition, the solution dissolves a minute but uniform layer of magnesium from the surface of the work piece and thereby removes any impurities which may be embedded in the surface of the metal. By treatment of magnesium work pieces as described herein, the magnesium surface is not only cleaned of its impurities but also is left bright and shiny. The bright and shiny surface thereby provided usually is smooth and mirror-like; but in some instances when certain alloys are treated, the surface, while still bright and shiny, may be slightly but uniformly roughened.

Because of its capacity for removing foreign substances and oxide and for dissolving embedded matter from magnesium surfaces, the process of my invention is especially adapted for the treatment of magnesium articles which have become coated with lubricants and various surface impurities and into which foreign matter has become embedded during working operations. However, the use of my process is not restricted to material which has been previously worked and it also may be used to brighten the surfaces of magnesium articles which have already been cleaned by other operations.

The following examples are given by way of illustration to show the operation of my cleaning and brightening process:

#### Example 1

A specimen of a magnesium base alloy nominally containing 4.0 per cent aluminum and 0.3 per cent manganese was cut from a sheet of the alloy as it came from a rolling operation, and, without being cleaned of lubricant and other foreign impurities, was immersed for 3 minutes at room temperature in 100 cc. of an aqueous solution containing 3 per cent by weight sulfuric acid and 3 per cent phenol. Upon removal from the solution, the specimen was found to have

been cleaned of its coating of lubricant and other foreign material, and to have a uniformly bright shiny surface.

#### Example 2

- 5 A test specimen similar to that described in Example 1, and of the same alloy, was treated at room temperature for 5 minutes in an aqueous solution containing 3 per cent sulfuric acid and 0.5 per cent pyrogallol. By this treatment, the lubricant and other foreign matter were removed and the surface of the specimen was left very smooth and bright.

#### Example 3

- 15 A specimen taken from a rolled sheet of commercially pure magnesium was immersed in an aqueous solution containing 3 per cent sulfuric acid and 3 per cent resorcinol at a temperature of about 30° C. At the end of about 3 minutes 20 the surface of the specimen was found to be free from foreign matter and to be mirror bright.

#### Example 4

- 25 A panel taken from a rolled sheet of commercially pure magnesium was immersed at room temperature for 1 minute in an aqueous solution containing 3 per cent sulfuric acid and 1 per cent gallic acid. The panel was thereby cleaned of all foreign matter and its surface left smooth 30 and mirror bright.

#### Example 5

- 35 Following immersion for 3 minutes of a rolled specimen of a magnesium base alloy containing 4.0 per cent aluminum and 0.3 per cent manganese in an aqueous solution containing 3 per cent sulfuric acid, 1 per cent phenol, and 2 per cent resorcinol, the specimen was found to have been 40 cleaned of foreign matter and to have a smooth bright surface.

#### Example 6

- 45 A specimen taken from a rolled sheet of commercially pure magnesium was immersed in an aqueous solution containing 3 per cent sulfuric acid, 1 per cent phenol, 2 per cent resorcinol, and 1 per cent pyrogallol at about room temperature. After treatment in this solution for about 3 minutes, the surface of the specimen was found to 50 be free from foreign matter and to be exceptionally bright and shiny.

55 These examples are given to indicate the compositions and methods of operating the solutions used in the practice of my invention, and it will be understood that variations in its practice are possible within the scope of the appended claims.

I claim:

- 60 1. The method of cleaning magnesium articles which comprises subjecting said articles to the action of an aqueous solution containing from about 1 to about 10 per cent sulfuric acid and a total of from about 0.5 to about 15 per cent of at least one soluble aromatic compound selected from the group consisting of phenol, resorcinol, 65 pyrogallol, and gallic acid.

- 65 2. The method of cleaning magnesium articles which comprises subjecting said articles to the action of an aqueous solution containing from about 2 to about 6 per cent sulfuric acid and a total of from about 3 to about 5 per cent of at least one soluble aromatic compound selected from the group consisting of phenol, resorcinol, pyrogallol, and gallic acid.

- 70 3. The method of treating wrought magnesium articles in order to remove lubricants and other

146

2,287,049

3

impurities therefrom and to produce a bright shiny surface thereupon, which method comprises subjecting said articles to the action of an aqueous solution containing from about 1 to about 10 per cent sulfuric acid and a total of from about 0.5 to about 15 per cent of at least one soluble aromatic compound selected from the group consisting of phenol, resorcinol, pyrogallol, and gallic acid.

4. The method of cleaning magnesium articles and producing a bright shiny surface thereupon which comprises subjecting said articles to the action of an aqueous solution containing from about 1 to about 10 per cent sulfuric acid and from about 0.5 to about 15 per cent phenol.

5. The method of cleaning magnesium articles and producing a bright shiny surface thereupon which comprises subjecting said articles to the action of an aqueous solution containing from about 1 to about 10 per cent sulfuric acid and from about 0.5 to about 15 per cent resorcinol.

6. The method of cleaning magnesium articles and producing a bright shiny surface thereupon which comprises subjecting said articles to the action of an aqueous solution containing from about 1 to about 10 per cent sulfuric acid and from about 0.5 to about 15 per cent pyrogallol.

15

MIKE A. MILLER.